

## UNITED STATES PATENT OFFICE

MILTON O. SCHUR AND BENJAMIN G. HOOS, OF BERLIN, NEW HAMPSHIRE, ASSIGNEES  
TO BROWN COMPANY, OF BERLIN, NEW HAMPSHIRE, A CORPORATION OF MAINE

## NITROCELLULOSE MANUFACTURE AND CELLULOSE THEREFOR

No Drawing.

Application filed April 20, 1931. Serial No. 531,638.

The subject of this invention is nitrocellulose manufacture and cellulose intended for such purpose, one of its primary objects being to provide cellulosic material in a form making for uniform and high quality nitrocellulose products.

It is the practice to nitrate cellulose fiber in a variety of physical conditions. In the case of chemical wood pulp, it is sometimes preferred to nitrate the pulp as it is purchased, for instance, in the form of thick sheets of dry pulp, known in the trade as "drier sheets". Such sheets may be nitrated by steeping in suitable nitrating acid com-

erably also the basis weight of thickness of the sheets. Thus, we have found that if the compactness is too high, the pores or void spaces in the sheets are so small that penetration of the quite viscous nitrating acid into and through the sheets, as well as the diffusion of the acid from the sheets into the main body of nitrating acid is greatly hindered, with the result that complete nitration of the sheets is prolonged and there is a tendency toward hydrolysis and other side reactions, with accompanying loss in yield and impairment in quality of the product. On the other hand, if the compactness is too low, retention of the expensive nitrating acid by the sheets becomes excessive; and the nitrating reaction may proceed so quickly as to generate heat to a point where hydrolysis and other side reactions also become excessive, especially when no provision is made to cool the batch undergoing nitration. From the standpoint of handling, the basis weight or thickness of the sheets is a factor of great importance. For instance, if the basis weight is too low, it is expensive to rack or otherwise handle the sheets for the nitrating and subsequent operations. In such a case, also, it is difficult to arrange the sheets in the bath of nitrating acid in such a way as to avoid undue contact between sheets, with a reasonably low ratio of nitrating acid to cellulose. Again, the sheets are flimsy and tend to move around in the bath of nitrating acid, as well as in the subsequent drowning, washing, and stabilizing baths. On the other hand, if the basis weight is too high, an inordinate time period is required for nitration of the sheets throughout; and this means tie-up of nitrating acid and nitrating equipment, and low-capacity production.

After considerable experimentation, we have established that optimum results are realized when drier sheets having a compactness between about 40 and 70 constitute the raw material undergoing nitration, particularly when such compactness is coordinate with a sheet thickness of about .040 to .070 inches. The sheets employed are preferably composed of refined wood pulps of high whiteness and high alpha cellulose content,

The pulp manufacturer produces drier sheets on a machine of the papermaking type, comprising a "wet end", to which the pulp is delivered and sheeted on a mould or Fourdrinier wire, and a "dry end" or series of drum driers, over which the sheet passes and is progressively dried. The sheet is usually made as compact as is possible, by press-rolls at the wet end of the machine acting to squeeze the maximum amount of water from the freshly-formed web, since otherwise there is added steam consumption and/or a reduction in the capacity of the machine. In fact, drier sheet as heretofore made normally had a compactness of about 70. The compactness value herein given represents the ratio of basis weight to 100 times the thickness of sheet in inches. The basis weight is the weight in pounds of 415,000 square inches of the sheet. According to this definition of compactness, the compactness value of a sheet having a basis weight of 240 pounds and an average thickness of .040 inches will be

$$\frac{240}{.040} \times 10^{-2}$$

or 60.

In our work on the nitration of drier sheets, we have discovered that for best and for consistent results it is essential to control the compactness of the sheets and pref-

such as are adapted for conversion into nitrocelluloses of a quality on a par with these derived from cotton. These wood pulps, in accordance with usual practice, may be used 5 in substantially unbeaten condition in the formation of the waterleaf sheets (i. e. sheets free from sizing materials or fillers). In the case of hardwood pulps e. g., birch, maple or poplar, the compactness of the sheets with- 10 in the range specified may be somewhat higher than in the case of soft-wood pulps, such as spruce. Our explanation for this is that, owing to the shorter lengths of the hardwood fibers, there is less chance for higher local 15 compactness in the sheets. In this connection, it is to be observed that in the formation of the sheet, the substantially unbeaten pulp is generally picked up as a layer on a cylinder mould, and is then passed through press- 20 rolls which dewater the layer as far as possible. Owing to the substantially unbeaten condition of the fibers, they are laid down "wildly" or as fiber aggregates, with the result that when the layer is passed between the 25 press-rolls, it receives an uneven pressure, the intensity of which is greatest, of course, where the layer is densest. This produces local areas in the sheet of very high compact- 30 ness, so that, although the average compact- ness of the sheet is, say, 70, there may be localities in the sheet where the compactness is considerably greater. This variation in local compactness of the sheet should be com- 35 batted by an intelligent operation of the wet end of the pulp drier, or be offset by a lower average compactness in the case of soft-wood pulps than in the case of hardwood pulps. The use of large volumes of water in the vat of the cylinder mould along with the pulp, 40 or the use of a Fourdrinier wet end, is of assistance in attaining uniform formation in the sheet, even though there is a tendency for soft-wood pulps to form "wilder" sheets than hardwood pulps. 45 The simplest method for controlling compactness to produce sheets such as we desire, is through adjustment of the press-rolls at the wet end of the machine, to exert less pressure on the wet sheet. Heretofore, as 50 already observed, it has been the practice to exert as much pressure as possible on the wet sheet, without crushing it, in order that the amount of water retained by the sheet entering the dry end of the machine be a minimum. The inevitable result of the applica- 55 tion of such high pressure is a drier sheet of relatively high compactness, usually above 70. We have found, however, that in the case of drier sheet intended for conversion into nitrocellulose, the higher steam consump- 60 tion and/or loss of production capacity resulting from the exertion of less pressure on the wet sheet is more than compensated for by the benefits received in the nitration process. The raising of the press-rolls on the

pulp drier can without trouble be made such that a dry sheet having a compactness between about 40 and 70 comes off the machine. Specifically, we prefer to produce drier sheets of a compactness of about 50, 70 although this compactness value may be departed from within the range specified, while still being within the ambit of the present invention.

The improvement in the nitrating process 75 realized by following the principles of the present invention obtains in the case of various compositions or nitrating acid. For example, we have performed nitrations in typical nitrating acid whose composition was 80 18% water, 22% nitric acid, and 60% sulphuric acid. When using drier sheets having a compactness of 48 and a thickness of .050 inches with such acid, the results obtained were notably better than those secured under similar conditions with drier sheets having a compactness of 75 and a thickness of .050 inches, or with drier sheets having a compactness of 75 and a thickness greater or less than .050 inches. In fact, the 85 nitrations performed with our sheets of lower compactness were completed sooner. Important, too, was the fact that the nitrated sheets obtained from our drier sheets of lower compactness lend themselves, after wash- 90 ing and stabilizing, to easier dehydration and to subsequent disintegration and solution or colloidization. Evidently, the greater porosity in the sheets endures after the 95 nitrating operation and permits a more rapid 100 displacement of the water in the sheets by alcohol, as well as a more rapid penetration of the solvent or colloidizing agent. Or, when the nitrated sheets are disintegrated, 105 as in a beater, they are less resistant to being pulled apart into shreds or pulp. The foregoing advantages also accrue when drier sheets of a compactness of 48 and a thickness of .050 inches are subjected to other nitrating processes, for instance, the multiple- 110 stage nitration process disclosed in application Serial No. 451,995, filed May 13, 1930, by Milton O. Schur. In such case, the first-stage nitrating acid may have a sulphuric to nitric acid ratio of less than 2 to 1, and the 115 second-stage nitrating acid may be one in which this ratio is greater, as in the usual nitrating acid. Thus, the primary-stage nitrating acid may be composed of 18.7% water, 40.6% nitric acid, and 40.7% sulphuric acid; and the secondary-stage nitrating acid may be composed of 18.7% water, 20.5% nitric acid, and 60.8% sulphuric acid. The 120 nitrocelluloses thus produced yield solutions of remarkable clarity and freedom from unnitritated fibers.

Our invention has its greatest utility, so far as we are now aware, in the field of chemical wood pulps, and more especially wood pulps of high whiteness and alpha 130

cellulose content intended for nitration purposes. Under certain economic conditions, it may be permissible to mix in a certain percentage of cotton linters with the wood fibers  
5 to make easier the attainment of low compactness sheets, for cotton linters tend to keep a sheet of mixed fibers bulky and porous. When in the appended claims we speak of "wood pulp" or "wood fibers", we, therefore,  
10 mean such fibrous material alone or blended with a subordinate proportion of, say 5% to 10%, more or less, cotton fibers.

What we claim is:

- 15 1. A process which comprises nitrating sheets of cellulose pulp whose thickness lies between .020 inches and .070 inches, and whose compactness in terms of ratio of basis weight to 100 times the thickness in inches lies between 40 and 70.
- 20 2. A sheet of interfelted wood fibers of high alpha cellulose content whose thickness lies between .020 inches and .070 inches, and whose compactness in terms of ratio of basis weight to 100 times the thickness in inches lies between 40 and 70.
- 25 3. A sheet of substantially unbeaten, interfelted wood pulp fibers of high whiteness and alpha cellulose content, whose thickness lies between .020 inches and .070 inches, and whose compactness in terms of ratio of basis weight to 100 times the thickness in inches lies between 40 and 70.

In testimony whereof we have affixed our signatures.

35 MILTON O. SCHUR.  
BENJAMIN G. HOOS.

40

45

50

55

60

65